

## UNITED STATES PATENT OFFICE

2,325,410

## REFINING OF ROSIN AND ROSIN DERIVATIVES

Donald A. Lister, Brunswick, Ga., assignor to Hercules Powder Company, Wilmington, Del., a corporation of Delaware

No Drawing. Application January 9, 1941,  
Serial No. 373,803

7 Claims. (Cl. 260—111)

This invention relates to the refining of rosin and rosin derivatives and more particularly to the treatment of impure or dark-colored rosin with furfural. Rosin has been heretofore refined by forming a solution thereof in a light petroleum distillate followed by selective solvent extraction of the solution with furfural which exerts a selective solvent action upon the rosin color bodies. Following this extraction step, the solution of refined rosin was evaporated to remove the petroleum distillate and leave a residue of refined rosin. The extract was also evaporated to remove the furfural and leave a residue of dark rosin. An example of such a rosin refining procedure is that described in the Kaiser and Hancock Patent No. 1,715,085 wherein the light petroleum distillate used is gasoline. In the procedure described in that patent, the mixture of furfural, gasoline, and rosin separates into two phases; one phase rich in furfural but containing some dissolved gasoline and also containing the rosin color bodies; the other phase rich in gasoline but containing some dissolved furfural and containing the pale rosin. A major difficulty connected with this prior rosin refining process is that the selective action of the system is diminished by solution of furfural in the gasoline phase and of gasoline in the furfural phase, each phase reaching saturation with respect to the chief ingredient of the other phase. The result is a reduced efficiency with which dark-colored and undesirable ingredients of the rosin are separated from light-colored ingredients, since the solubility of the solvents in each other diminishes the dissimilarity of the phases. Accordingly, the efficiency of the separation is likewise diminished, the dark-colored and undesirable ingredients being appreciably soluble in the gasoline phase.

An object of the present invention is to devise a process whereby rosin of a given color grade can be obtained more economically and more efficiently or whereby rosin of a paler color grade may be produced. Another object is to provide a process for refining rosin which gives an improved yield of product. Other objects will more fully hereinafter appear.

I have discovered that by the introduction to the mixture of furfural, light petroleum distillate such as gasoline, and rosin or the like, of water to the extent of more than 1% by weight based on the weight of the furfural and water, the furfural and light petroleum distillate dissolve to a lesser extent in one another so that either a paler grade of refined rosin or a higher yield

of rosin of a given color, or a higher yield of a paler grade may be obtained. Preferably, this is accomplished by dissolving water in the furfural to be employed, to the extent of more than 1% by weight based on the weight of furfural and water. However, though less preferably, water may be added to the mixture of anhydrous or substantially anhydrous furfural, gasoline, and rosin, whereupon water will dissolve in the furfural phase, increasing the selective distribution of the rosin ingredients between the two phases. The amount of water may range up to the saturation point of the furfural at ordinary atmospheric temperatures (15 to 25° C.). If desired, an excess of water may be present, although such excess forms a third phase and has no effect in the process other than to maintain the furfural saturated with water. In general, the presence of a third phase of water is undesirable because of mechanical difficulties introduced in connection with the separation of the phases from one another.

The light petroleum distillate employed in the process of the present invention may be any light mobile petroleum distillate capable of yielding a rosin solution of high concentration but of low viscosity. In general, any petroleum distillate having a boiling point range not above that of kerosene may be utilized. For example, I may use petroleum ether (boiling range 40–60° C.), petroleum spirit (boiling range 80–130° C.), V. M. & P. naphtha (boiling range 100–160° C.), mineral spirit (90% below 200° C.), gasoline such as that suitable for use in spark fired internal combustion motors (having an initial boiling point of from about 21° C. up to about 60° C. and an end boiling point of from about 177° C. to about 232° C.). I may use gasoline having a higher initial boiling point such as, for example, an initial boiling point of 93° C., which is unsuitable for use as motor fuel, but which is termed gasoline in the industry. I may use Stoddard solvent (50% or more below 177° C., end point not higher than 210° C.), or I may use kerosene which has a boiling range of 150–270° C. I may likewise use any of the foregoing light petroleum distillates which has been treated with furfural, sulfur dioxide, sulfuric acid, chlorosulfonic acid, selective adsorbents such as clay, etc. for removal of nonparaffin constituents. It is preferred, however, to use light petroleum distillate of the type commercially referred to in the industry as gasoline. In general, it is preferred to use light petroleum distillate boiling not above 200° C., preferably par-

affinic in character and having a critical solution temperature in aniline not lower than 60° C.

The process of the present invention is particularly suitable for refining rosin containing visible or latent color bodies, for example, wood or gum rosin. Instead of rosin, equivalent materials such as the rosin acids such as commercial abietic acid, pimamic acid, sapinic acid, etc. may be treated. The invention is also suitable for refining rosin derivatives such as modified rosins such as rosin which has been treated with a hydrogenating catalyst in the absence of hydrogen and known as "Hyex" rosin, hydrogenated rosin, polymerized rosin, isomerized rosin, heat treated rosin, etc., rosin esters such as ester gum, esters of rosin with methanol, ethanol, propanol, butanol, amyl alcohol, cetyl alcohol, lauryl alcohol, stearyl alcohol, furfuryl alcohol, abietanol, phenol, benzyl alcohol, etc. or with polyhydric alcohols such as ethylene glycol, diethylene glycol, triethylene glycol, glycerol, erythritol, pentaerythritol, sorbitol, mannitol, etc., where such rosin derivatives contain visible or latent color bodies. The invention is also applicable to esters of modified rosins such as esters of "Hyex" rosin, hydrogenated rosin, polymerized rosin, etc. Similarly, the invention is suitable for the refining of rosin alcohols and hydrogenated rosin alcohols such as are obtained by reducing the rosin acid carboxyl group to a hydroxyl (e. g. abietic acid to abietanol), etc., and organic esters of such rosin alcohols, and other rosin derivatives of like nature where such derivatives contain visible or latent color bodies.

The process of the present invention comprises commingling light petroleum distillate such as gasoline, rosin or the like, furfural, and water in any manner which will result in the formation of separable phases; the one phase rich in furfural and containing dissolved therein the rosin color bodies, a small amount of dissolved petroleum distillate, and water, preferably in amount approaching or equaling the solubility of water in the furfural phase; the other phase being rich in gasoline and containing a small amount of dissolved furfural, light colored rosin or the like, and only a trace of dissolved water. Excess water, if present in slight excess so as to form a third separate phase, does not affect the refining process.

It is preferred to dissolve the rosin or the like in the light petroleum distillate such as gasoline to the extent of from about 10 to about 40% of rosin by weight based on the weight of rosin and gasoline. A convenient concentration is 20% by weight. The amount of furfural may range from about 50% to about 150% by weight based on the weight of rosin taken, depending upon the extent of coloration of the rosin, and numerous other factors. A preferred procedure is to maintain the mixture at an elevated temperature sufficient to render it homogeneous, followed by cooling the mixture to 25° F. or below, separation of the furfural phase from the gasoline phase, and recovery from the respective phases of the resinous components dissolved therein.

The following specific examples show typical methods of carrying out the present invention.

#### EXAMPLE 1

A solution comprising 850 parts by weight of gasoline and 150 parts by weight of dark-colored rosin was passed upwardly through a packed tower, a solution comprising 106 parts by weight

of anhydrous furfural and 4 parts by weight of water being passed downwardly through the tower in a countercurrent relationship. The furfural phase dissolved from the gasoline phase

5 a portion of the rosin very dark in color. The furfural phase was discharged at the bottom, the furfural and water evaporated and recycled, the gasoline layer containing a portion of the original rosin which was very light in color was discharged at the top of the tower and evaporated, the recovered gasoline being recycled. An identical run wherein 106.8 parts by weight of technical furfural containing 0.75% of water was employed instead of the mixture of 106 parts 10 of anhydrous furfural and 4 parts of water, gave a materially darker refined rosin in a lower yield. A further run wherein 106 parts by weight of anhydrous furfural was employed instead of furfural containing water gave a still lower yield 15 of a still darker refined rosin.

#### EXAMPLE 2

Three hundred grams of solution comprising 50 g. of FF wood rosin in 250 g. of gasoline was placed in a separatory funnel and 45 g. anhydrous furfural and 1 g. water were added, the mixture shaken vigorously and allowed to stand whereupon a 26 g. dark layer was separated off. The residual gasoline layer was treated again with 23 g. anhydrous furfural and 1 g. water, whereupon a 36 g. dark layer was separated off. The gasoline layer remaining was evaporated and a 79% yield of rosin grading I in color was recovered.

Further evidence of the effect of dissolved water in the furfural employed upon the color grade and yield of purified rosin is indicated in the following table of runs, in each of which 300 g. of a solution of 50 g. of FF wood rosin in gasoline 35 was contacted with the indicated amount of anhydrous furfural containing the indicated amount of water, the residual gasoline phase being separated and again washed with anhydrous furfural containing water as indicated under "second wash."

Table 1

|                                                     | Example No. |          |          |          |
|-----------------------------------------------------|-------------|----------|----------|----------|
|                                                     | 3 (blank)   | 4        | 5        | 6        |
| 50                                                  |             |          |          |          |
| First wash:                                         |             |          |          |          |
| Anhydrous furfural                                  |             |          |          |          |
| -----cubic centimeter-----                          | 40          | 40       | 30       | 30       |
| Water-----do-----                                   | None        | 1.0      | 1.0      | 1.0      |
| Wt. % of water (based on wt. of furfural and water) | 0.0         | 2.1      | 2.8      | 2.8      |
| Volume of furfural layer separating                 |             |          |          |          |
| -----cubic centimeter-----                          | 8.5         | 23.0     | 10.2     | 10.5     |
| Second wash:                                        |             |          |          |          |
| Anhydrous furfural                                  |             |          |          |          |
| -----cubic centimeter-----                          | 20          | 20       | 20       | 14       |
| Water-----do-----                                   | None        | 1.0      | 1.0      | 0.7      |
| Wt. % of water                                      | 0.0         | 4.1      | 4.1      | 4.1      |
| Volume of furfural layer separating                 |             |          |          |          |
| -----cubic centimeter-----                          | 29.7        | 32.0     | 29.6     | 18.0     |
| Results-refined rosin                               |             |          |          |          |
| Yield-----per cent-----                             | 86.8        | 78.5     | 85.2     | 87.6     |
| Lovibond color, Amber+Red                           | 80+8.5 G    | 80+1.0 I | 80+3.7 H | 80+6.0 G |
| Rosin color grade                                   |             |          |          |          |

Examples 3 and 4 show that where equal quantities of furfural are used, the addition of water results in a considerably paler rosin, namely a rosin of 7.5 less red and two color grades higher. The slightly lower yield is explained by considering the volumes of dark furfural layer separating off in the first wash. In the presence of 2.1% of water less furfural dissolved in the gasoline

layer, and so there was a larger furfural layer present in which the rosin color bodies could dissolve. By extracting this separated furfural phase with fresh gasoline, it was found that a considerable amount of pale rosin could be recovered therefrom.

In Example 5, the volume of furfural-water washes was reduced to the point where a yield comparable with the blank Example 3 was obtained. Yet the rosin recovered had a color one grade above that yielded by the blank and Lovibond color lower by 4.8 red.

In Example 6, the volume of furfural-water washes was reduced still further, giving a higher yield of purified rosin than the blank, and a purified rosin of a color of 2.5 red lower than the purified rosin of the blank. The procedure of this example therefore resulted in both higher yield and improved color.

The anhydrous furfural employed in the foregoing examples was prepared from technical furfural containing 0.75% water by first vacuum distilling, and then heating in a 100-105°C. oil bath at 50-60 mm. absolute pressure with carbon dioxide bubbling up through the furfural until the distillate contained no moisture.

I have still further discovered that improved results may be obtained by using furfural containing more than 1% by weight of water in the preparation of a substantially petroleum-hydrocarbon insoluble resin from the total resinous extract from pine wood obtained with an aromatic hydrocarbon such as benzene. For example I may dissolve such a total resinous extract (left upon evaporation of the benzene) in a light petroleum hydrocarbon such as gasoline at an elevated temperature, add with stirring furfural containing more than 1% of water in an amount equal to say one-third of the weight of the crude resin taken, to cause dissolution of that portion of the resinous extract which is substantially insoluble in light petroleum hydrocarbons at room temperature, and effect separation of the furfural phase, leaving a gasoline solution of impure rosin (FF grade) as the raffinate. I may then advantageously extract the impure rosin solution or raffinate with fresh furfural containing more than 1% of water in the manner set forth above in detail. In this way, I effect a better separation of the petroleum-insoluble resin prior to the refining of the crude rosin.

In the procedure just described I may agitate the crude total resinous extract with a mixture of the gasoline and the furfural containing more than 1% of water, instead of first dissolving the extract in gasoline. Likewise, I may effect the inter-mixture and commingling of the crude total extract, the gasoline, and the furfural containing more than 1% of water, at an elevated temperature which may or may not be sufficiently high to bring about miscibility, followed by cooling to separate the phases.

Following are examples showing the combined procedure just described.

#### EXAMPLE 7

The total benzene extract of pine wood (known as "FF No. 3 rosin" and comprising a mixture of FF wood rosin and the petroleum hydrocarbon-insoluble resin) had the following analysis:

Acid number 144

Melting point 177°F.

Specific rotation +14.8°

Color (Lovibond) 80 Amber+175 Red

Gasoline-insoluble 16.3%

Seventy-five grams of the foregoing resin was dissolved in 75 g. of narrow range gasoline (B. R. 200-270°F.) by heating until solution of the gasoline-soluble constituents was obtained. The gasoline-insoluble constituents of the resin remained in suspension. The solution was diluted with 175 g. of additional narrow range gasoline of suitable temperature to give 325 g. of solution at 90-95°F.

- To this solution there was added with rapid stirring a solution consisting of 25 g. of anhydrous furfural and 0.5 g. of water. The addition of this caused solution of the more insoluble portion of the gasoline-insoluble constituents of the crude resin by forming a lower furfural layer containing those constituents. The mixture was maintained at about 90°F. during this step. The upper gasoline layer of partially refined rosin (FF) at 90°F. was then decanted off.
- To this gasoline layer of FF rosin there was added 60 g. of anhydrous furfural in admixture with 1.2 g. of water (dissolved therein), with agitation at about 85°F. for 5 minutes. The mixture was then allowed to settle whereupon the lower furfural layer of impurities and color bodies was drawn off. The refined rosin solution (the upper layer) was evaporated to recover the refined rosin. There was obtained a yield of 47.3 g. of refined rosin having a color of H<sub>7</sub> on the photoelectric scale based on the U. S. Government rosin standard. This was a yield of 63.7% of the original crude extract.

#### EXAMPLES 8 TO 10

- Example 7 was duplicated exactly except that the amount of water based on the weight of furfural and water was progressively increased and the amount of furfural and water used for refining the gasoline layer left after the first extraction was progressively diminished so as to give the same color of refined rosin. In this way direct comparison of the yields of refined rosin of a given color grade was possible. The conditions and results are set forth in the following Table II wherein there have also been tabulated Example 7 and a comparative run using no water (the top run in Table II).

Table II

| Example               | Per cent of water based on weight of furfural and water | Ratio of anhydrous furfural to original crude resinous extract |                      | Refined rosin |                |
|-----------------------|---------------------------------------------------------|----------------------------------------------------------------|----------------------|---------------|----------------|
|                       |                                                         | In first extraction                                            | In second extraction | Yield         | Color          |
|                       |                                                         | Per cent                                                       | Per cent             |               |                |
| Blank comparative run | 0.0                                                     | 33 1/3                                                         | 133 1/3              | 59.2          | H <sub>7</sub> |
| 7                     | 1.96                                                    | 33 1/3                                                         | 79 2/3               | 63.7          | H <sub>7</sub> |
| 8                     | 2.91                                                    | 33 1/3                                                         | 66 2/3               | 65.0          | H <sub>7</sub> |
| 9                     | 3.84                                                    | 33 1/3                                                         | 47.9                 | 66.5          | H <sub>7</sub> |
| 10 <sup>1</sup>       | 4.75                                                    | 33 1/3                                                         | 47.6                 | 67.3          | H <sub>7</sub> |

<sup>1</sup> Solution of the water in the furfural in this run was obtained by heating the mixture of furfural and water to about 100°C. During the second extraction some of this water was thrown out as droplets in the furfural layer.

The anhydrous furfural used in the runs tabulated in the foregoing Table II was prepared by distilling fresh technical furfural rejecting the first 20% over and retaining the next 60% over for use.

Examination of the foregoing Table II shows a marked advantage of the present invention in that the amount of furfural used for refining the impure (FF) rosin may be greatly reduced and yet a higher yield of refined rosin of a given

color grade is produced. The table further illustrates that there is but little improvement in refining effect in going from 3.84% of water to 4.76%.

#### Color grading

In the foregoing Table II, the color of the refined rosins were determined on a photoelectric grader which is more accurate than the Lovibond tintometer method. With this method of grading each of the Lovibond color grades is divided into eight divisions so that colors are reported in eighths of a grade. In Table II the amount of furfural used in the refining of the impure rosin (i. e., the second extraction) was progressively reduced so as to give a rosin of color H<sub>7</sub>, thereby enabling the yields to be directly compared. The next color division above H<sub>7</sub> is "I."

The amount of water dissolved in the furfural may vary upwardly from 1% by weight of the furfural and water to saturation at atmospheric temperature. Preferably, at least about 2% of water is employed. The higher the amount of water, the better the results. Use of furfural saturated at the temperature at which phase separation is effected with water is particularly advantageous and convenient. Furfural will dissolve water to a 4.8% solution at 20° C.

From the foregoing, it will be seen that the process of the present invention gives rise to numerous advantages over the prior art process of refining rosin with furfural, among these advantages being the improved yield of light-colored rosin which is obtainable with the process of the invention. Numerous other advantages of the process will be apparent to those skilled in the art.

It will be understood that the details and examples hereinbefore set forth are illustrative only and that the invention as broadly described and claimed is in no way limited thereby.

What I claim and desire to protect by Letters Patent is:

1. The method of refining a rosiny material selected from the group consisting of rosins, rosin acids, rosin esters, rosin alcohols, and esters of rosin alcohols which comprises treating a solution of said material in a light petroleum distillate with furfural having water dissolved therein in an amount ranging from above 1% to saturation at atmospheric temperature, separating the furfural phase from the petroleum distillate phase containing purified rosin, and recovering from the two phases the resinous components dissolved therein.

2. The method of refining a rosiny material selected from the group consisting of rosins, rosin acids, rosin esters, rosin alcohols, and esters of rosin alcohols which comprises treating about a 10% to about a 40% by weight solution of said material in a light petroleum distillate with furfural in an amount ranging from about 50% to about 150% by weight based on the weight of rosiny material in said solution, said furfural having water dissolved therein in an amount ranging from above 1% to saturation at atmospheric temperature, separating the furfural phase from the petroleum distillate phase containing purified rosin, and recovering from the two phases the resinous components dissolved therein.

3. The method of refining a rosiny material selected from the group consisting of rosins,

rosin acids, rosin esters, rosin alcohols, and esters of rosin alcohols which comprises treating about a 10% to about a 40% by weight solution of said material in a light petroleum distillate with furfural in an amount ranging from about 50% to about 150% by weight based on the weight of rosiny material in said solution, said furfural having water dissolved therein in an amount ranging from above 1% to saturation at atmospheric temperature, maintaining the mixture at an elevated temperature sufficient to render it homogeneous, and then separating the furfural phase from the petroleum distillate phase containing purified rosin, and recovering from the two phases the resinous components dissolved therein.

4. The method of refining a rosiny material selected from the group consisting of rosins, rosin acids, rosin esters, rosin alcohols, and esters of rosin alcohols which comprises treating about a 10% to about a 40% by weight solution of said material in a light petroleum distillate with furfural in an amount ranging from about 50% to about 150% by weight based on the weight of rosiny material in said solution, said furfural having water dissolved therein in an amount ranging from above 1% to saturation at atmospheric temperature, maintaining the mixture at an elevated temperature sufficient to render it homogeneous, cooling the mixture at least to 25° F., and then separating the furfural phase from the petroleum distillate phase containing purified rosin, and recovering from the two phases the resinous components dissolved therein.

5. The method of refining rosin which comprises contacting about a 10% to about a 40% by weight solution thereof in gasoline with furfural in an amount ranging from about 50% to about 150% by weight based on the weight of rosin in said solution, said furfural having water dissolved therein in an amount ranging from about 1% to saturation at atmospheric temperature, maintaining the mixture at an elevated temperature sufficient to render it homogeneous, cooling the mixture at least to 25° F., separating the gasoline and furfural phases, and recovering the rosin dissolved in said phases.

6. The method of refining a rosin ester which comprises treating about a 10% to about a 40% by weight solution thereof in gasoline with furfural in an amount ranging from about 50% to about 150% by weight based on the weight of rosin ester in said solution, said furfural having water dissolved therein in an amount ranging from above 1% to saturation at atmospheric temperature, maintaining the mixture at an elevated temperature sufficient to render it homogeneous, cooling the mixture at least to 25° F., separating the gasoline and furfural phases and recovering the rosin ester dissolved in said phases.

7. The method of refining a total aromatic extract of pine wood which comprises contacting about a 10% to about a 40% by weight solution thereof in gasoline with furfural in an amount ranging from about 50% to about 150% by weight based on the weight of extract in said solution, said furfural having water dissolved therein in an amount ranging from above 1% to saturation at atmospheric temperature, and then separating the gasoline and furfural phases, and recovering the rosin dissolved in said gasoline phase.